

## UNITED STATES PATENT OFFICE.

GEORGE H. ELLIS, OF ST. PAUL, MINNESOTA.

## INSULATING BOARD AND PROCESS OF MAKING THE SAME.

No Drawing.

Application filed March 15, 1921. Serial No. 452,523.

*To all whom it may concern:*

Be it known that I, GEORGE H. ELLIS, a citizen of the United States, residing at St. Paul, in the county of Ramsey and State of Minnesota, have invented new and useful Improvements in Insulating Boards and Processes of Making the Same, of which the following is a specification.

My invention relates to improvements in insulating boards and particularly such boards as are molded or felted from vegetable fibres.

The object of my invention is to produce economically an efficient insulating board or block of fibrous material.

A further object is to provide such a board or block with a sizing and binder which is permanent and repellent to moisture.

20 A further object is to provide a foundation for stucco or plaster which will retain its rigidity and efficiency when exposed to the weather.

After extensive experiments I have discovered that it is possible to apply directly to the fibres of which such a board is composed, a bitumen such as asphalt or coal tar, during the process of pulping the material for such board, and that by so doing a 30 stronger and lighter product and one better adapted to form a foundation for stucco or plaster may be secured.

It has been common practice in paper making, as well as in the manufacture of insulating board, to use what is known as engine sizing such as rosin soap precipitated with aluminum sulphate, and to a less extent casein precipitated with a reagent, such as alum has been employed, but such sizings

40 cause deterioration of the product, particularly when it is exposed to moisture, and while this susceptibility may be of small importance where the product is paper used for ordinary purposes it is seriously detri-

45 mental to an insulating board which forms the foundation for plaster or is long exposed to the weather. Thus an insulating material in which aluminum sulphate and rosin soap have been used will in time deteriorate because of the detrimental effect 50 of these agents upon cellulose. The chemi-

cal changes which take place, gradually weaken and make brittle the product.

In manufacturing my insulating board I prefer to employ an ordinary paper maker's 5 beating engine. Water, preferably hot, together with cellular material such as waste paper, straw or wood fibres are placed in the beater in the usual proportions to form a pulp. I then add a bitumen such as coal tar 60 or asphalt in a fluid or semi-fluid state. Twelve to fifteen per cent of bitumen (by bulk) is sufficient. It is well known that tar, asphalt and other bitumens do not mix readily with water, and I, therefore, depend 65 upon the mechanical action of the beater cylinder, blades and concave to paint the fibres with the bitumen while the stock is being reduced to a pulp. After the fibres have been thoroughly coated with the bitumen, the stock is removed from the beater and drained, when it may be either felted or molded in the usual way and then dried. I have found that this process not only 70 water proofs the fibres themselves but reduces the capillary attraction which tends to carry moisture into the insulating board. I thus eliminate from my board all free precipitates which predispose the product to deterioration and substitute a material 75 which is cheaper and better suited to the purpose than the rosin size, alum or casein heretofore employed. In addition to being substantially water proof and having no tendency to soften when subjected to moisture my board has a greater number of caged air cells than boards made by processes heretofore known to me and it is, therefore, lighter and better adapted for insulating purposes. 80

Having described my invention what I claim as new and desire to protect by Letters Patent is:

1. The method of producing insulating board which consist in immersing fibrous stock in liquid bitumen and water, then agitating said materials, whereby the fibres are coated with bitumen and the stock is pulped, then molding or felting the stock 95 into a board and finally drying the same. 100

2. The method of producing insulating board which consist in first placing fibrous

stock in a beating engine in the presence of liquid bitumen and water, then beating said materials, whereby the individual fibres are coated with bitumen and the stock is simultaneously pulped, then molding or felting the stock into a board and finally drying the same.

3. A board composed of vegetable fibres

felted or molded with a binder of liquid bitumen, and constituting a porous, self sustaining body adapted to form a base for plaster. 10

In testimony whereof, I have hereunto signed my name to this specification.

GEORGE H. ELLIS.